

## UNITED STATES PATENT OFFICE

2,179,449

METHOD FOR THE MANUFACTURE OF  
CELLULOSE PRODUCTS

Johann Eggert, Berlin, and Walter Gellendien,  
Berlin-Charlottenburg, Germany, assignors to  
Deutsche Hydrierwerke Aktiengesellschaft, Ber-  
lin-Charlottenburg, Germany, a corporation of  
Germany

No Drawing. Application February 10, 1937, Se-  
rial No. 125,072. In Germany January 21, 1936

8 Claims. (Cl. 106—40)

It is known that cellulose materials of any form such as fibres, threads, ribbons, films, foils, plates, plastic masses and the like obtainable by precipitation from solutions of cellulose compounds such as 5 nitrocellulose, acetylcellulose, benzylcellulose, ethylcellulose, and particularly from aqueous xanthogenate cellulose solutions, are of a small strength in wet state which often shows with threads only 50 to 60% of the strength in dry state.

Now it has been found, that with cellulose products of regenerated cellulose obtainable from xanthogenate-cellulose-solutions or likewise from cellulose-derivatives, we are in a position to attain 15 an almost 100% wet strength (referred to the strength in dry state) in adding to the cellulose solutions, before working them up into the shaped material, furfural or its homologues or derivatives, and particularly alcoholic hydrogenation products of the furfural or their esters or ethers respectively.

Besides the furfural also e. g. the methyl-furfural, the furfuryl-alcohol, the tetrahydro-furfuryl-alcohol, the methyl-furfuryl-alcohol, are 25 to be considered. Further one may apply the ethers and esters of those compounds as far as they are of an alcohol character such as e. g. the furfuryl-acetate, the tetrahydro-furfuryl-benzoate, the methylfurfuryl adipic acid ester, the furfuryl-butyl ether, the tetrahydro-furfuryl-dodecyl ether, the methylfurfuryl-oleyl ether, the methylfurfuryl-monoglycerol ether. Generally speaking the hydroxyl groups of the aforesaid compounds of an alcoholic character may be alkoxylated or esterified by organic residues containing 30 1 to 18 carbon atoms and eventually further substituents such as hydroxyl-groups, amino-groups and the like.

Besides the afore-cited products we are also 40 allowed to co-employ other suitable substances such as naphthol, naphthol sulfonic salts, formaldehyde, carbamide and the like. For products made of aqueous xanthogenate-cellulose solutions there are, interalia, furfuryl-alcohol mixtures 45 with cresols such as meta- or para-cresol or their derivatives, which are likewise apt for the purpose in question.

The additional amounts of the means according 50 to the present invention are calculated on the amounts of cellulose or cellulose derivatives respectively present in these solutions and the respective proportion varies from approximate 0.2 to 10% but the most advantageous proportions lie between 0.5 and 2.5%.

## Example 1

To an aqueous cellulose-xanthogenate solution which is to contain 6 to 7% of cellulose and approximately 6% of alkali one adds, just before the beginning of the spinning process, 1% of hydrogenated furfuryl-alcohol in a watery dissolution. This cellulose-solution is, in an acid spinning-bath, shaped in the usual way into threads or into any other material. The after-treatment 10 is accomplished in the well-known manner in de-sulfurizing with sodium-sulfite and with subsequent washing, bleaching and finishing. The thus treated threads show a high wet strength of approximately 98% (referred to the dry 15 strength).

## Example 2

A mixture of 1 weight part of furfuryl-alcohol and 1 part of ortho- or meta- or para-cresol is added to an aqueous cellulose-xanthogenate-solution 20 at the rate of 1 to 2% (referred to dry cellulose). It is recommendable to dissolve the said product in a solvent that itself is soluble in water. The working up of the cellulose-solution into shaped goods is done in the usual way. A shaped lace made with this solution from regenerated cellulose shows an excellent wet strength.

## Example 3

To an aqueous cellulose-xanthogenate-solution 30 (viscose) of the usual concentration applied in the manufacture of cellulose hydrate films, one adds 2% of furfuryl-alcohol (referred to the cellulose) preferably in the form of an aqueous solution. The cellulose-xanthogenate-solution is 35 worked up in the well-known way into cellulose-hydrate-film on a film-pouring machine. The thus obtained film, when finished, is of an excellent fastness.

## Example 4

To an acetyl-cellulose solution in organic solvents of a concentration as usual in the manufacture of acetate-artificial silk, one adds 2% of purified furfural (calculated to acetyl-cellulose). This solution is spun in the usual manner. The 45 thus obtained acetate-silk shows, after the working up, an extraordinary strength especially in applying an extended warm-treatment e. g. during the drying-process.

We claim:

1. Cellulose articles consisting of regenerated cellulose containing furfuryl alcohol.
2. Cellulose articles consisting of regenerated cellulose containing mixtures of furfuryl alcohol and a cresol.

3. Cellulose article consisting of regenerated cellulose containing a compound of the group consisting of furfural, methyl furfural, furfuryl alcohol, methyl furfuryl alcohol, furfuryl acetate, methyl furfuryl adipic acid ester, furfuryl butyl ether, methyl furfuryl oleyl ether, methyl furfuryl monoglycerol ether.
4. Cellulose article consisting of regenerated cellulose containing a compound of the group consisting of furfural, methyl furfural, furfuryl alcohol, methyl furfuryl alcohol, furfuryl acetate, methyl furfuryl adipic acid ester, furfuryl butyl ether, methyl furfuryl oleyl ether, methyl furfuryl monoglycerol ether together with a compound of the group consisting of naphthol, naphthol sulfonic acid salts, and cresol.
5. Cellulose article consisting of regenerated

cellulose containing a compound of the group consisting of furfural, methyl furfural, furfuryl alcohol, methyl furfuryl alcohol, furfuryl acetate, methyl furfuryl adipic acid ester, furfuryl butyl ether, methyl furfuryl oleyl ether, methyl furfuryl monoglycerol ether together with formaldehyde.

6. Cellulose articles consisting of cellulosic material containing about 0.5 to 2.5% of the hydrogenation products of furfural.

7. Cellulose articles consisting of cellulosic material containing between 0.2 and 10% of hydrogenation products of furfural with a cresol.

8. Shaped articles consisting of regenerated cellulose containing hydrogenation products of furfural.

JOHANN EGGERT.  
WALTER GELLENDIEN.

5

10

15